

## UNITED STATES PATENT OFFICE

2,385,125

NITROCELLULOSE LACQUER  
COMPOSITIONS

Gerald R. Barrett, Winchester, Mass., assignor to  
Monsanto Chemical Company, St. Louis, Mo., a  
corporation of Delaware

No Drawing. Application December 31, 1942,  
Serial No. 470,907

9 Claims. (Cl. 106—181)

This invention relates to the treatment of lacquer compositions to prevent or substantially reduce the tendency of such compositions to gel or liver. More particularly it relates to the preparation of nitrocellulose lacquer compositions having a markedly decreased tendency to gel.

It is well known that nitrocellulose lacquers containing as pigments certain metal constituents, such as, bronze, aluminum-bronze, gold-bronze or other copper-containing powders or pastes, are subject to rapid gelation or livering. Moreover, these lacquers tend to become gelled or gelatinized in the presence of lead powders or pastes, and even in the absence of metal powders, when they are packaged in lead-lined or lead containers, such as collapsible tubes of lead foil.

It is accordingly a primary object of the present invention to provide inhibiting agents, which when added to nitrocellulose lacquers in small quantities will markedly reduce or completely prevent any tendency toward gel formation.

A further object of the invention is to provide an inhibiting agent of the type described which is more effective than most, if not all previously known inhibiting agents.

Still further objects and advantages of the invention will appear from the following description and appended claims. Before explaining in detail the present invention, however, it is to be understood that the invention is not limited in its application to the details described herein, since the invention is capable of other embodiments and of being practiced or carried out in various ways.

The invention is carried out in general by incorporating in the usual lacquer formulations, either containing bronze or other similar powders or intended to be packaged in lead lined or like containers, small amounts of a certain polycarboxylic organic acid. Although malic, citric, tartaric and other polycarboxylic organic acids have been used previously for this purpose, these acids are not as effective as the particular acid which is the subject of this invention.

According to this invention the most suitable polycarboxylic organic acid for obtaining maximum prevention or reduction in gelation is malic acid. This acid is so effective that it may sometimes be used in amounts as small as 0.01% by weight based on the weight of the clear or pigmented lacquer being treated. In general, however, it is preferable to employ amounts of the acid varying from 0.05 to 1% based on the lacquer solution, either pigmented or otherwise. In some cases, it is desirable to use amounts of acid as large as 5%, but in most instances concentrations as large as this are to be avoided, as these larger amounts have a tendency to crystal-

lize from the lacquer film and they also decrease the water resistance of the film.

In general the presence of copper or lead is the chief cause of gelation in nitrocellulose lacquers, that is bronzes or other metal powders high in copper or lead are most apt to cause gelation. For this reason, relatively large amounts of the malonic acid are usually required in the case of lacquers containing powders or pigments which are high in copper or lead. Only relatively small amounts of the malonic acid are required, on the other hand, in the case of clear lacquers which are subjected to the undesired action of metals merely by being packaged in metal containers, due to the considerably smaller surface area to which the lacquer is exposed in such instances.

A further understanding of the invention will be obtained from the following examples.

## Example I

20 A clear lacquer base of the following composition was first prepared:

|                                          | Per cent by weight |
|------------------------------------------|--------------------|
| Cellulose nitrate (1/2 second viscosity) | 25                 |
| 25 Butyl acetate                         | 31                 |
| Toluene                                  | 30.6               |
| Denatured alcohol                        | 13                 |
| Malonic acid                             | 0.4                |

30 Twelve parts of gold bronze were added to 100 parts of the above clear lacquer. Upon packaging samples of the clear lacquer and the bronze-containing lacquer, as well as samples of the above clear lacquer with the malonic acid omitted, in lead containers, it was found that the lacquers containing the malonic acid, either with or without addition of the gold bronze, were more resistant to gelation than similar lacquers which were free of malonic acid.

## Example II

40 A clear lacquer base of the following composition was first prepared:

|                           | Per cent by weight |
|---------------------------|--------------------|
| Celluloid scrap           | 15                 |
| 45 Acetone                | 36                 |
| Petroleum lacquer diluent | 14                 |
| Denatured alcohol         | 35                 |

50 To 100 parts of the above clear lacquer 1.5 parts of fine aluminum bronze paste and 15 parts of lead paste were added. In the absence of inhibitor the resulting composition gelled in a few minutes. Upon adding 0.15% of malic acid to the above paste-containing lacquer, the composition resisted gelation for two months, while gelation set in after only three days when an equal quantity of malic acid was employed. In the absence of the lead paste, but with the composition stored in a lead lined container the

above amount of malonic acid appeared adequate to prevent gelation indefinitely.

*Example III*

To 100 parts of a clear lacquer base having the following composition:

|                     | Per cent by weight |
|---------------------|--------------------|
| Celluloid scrap     | 15                 |
| Butyl acetate       | 15                 |
| Acetone             | 15                 |
| Methyl ethyl ketone | 25                 |
| Denatured alcohol   | 30                 |

were added 5 parts of copper lining powder. In the absence of inhibitor the above lacquer composition gelled in a few hours. Upon adding 0.1 part of malonic acid to an equal amount of the above powder-containing lacquer, the composition remained fluid after three months, while the addition of 0.1 part of malic acid to an equal amount of powder-containing lacquer only delayed gelation for three days.

Similar tests on a lacquer composition similar to the above but with lead paste substituted for the copper lining powder also indicated that malonic acid is superior to malic acid as an effective inhibitor of gelation.

*Example IV*

To a clear lacquer base having the following composition:

|                                       | Per cent by weight |
|---------------------------------------|--------------------|
| Nitrocellulose (15 seconds viscosity) | 8                  |
| Ethyl acetate                         | 10                 |
| Butyl acetate                         | 20                 |
| Butyl alcohol                         | 10                 |
| Ethyl alcohol                         | 10                 |
| Toluene                               | 34                 |
| Ester gum                             | 5                  |
| Dibutyl phthalate                     | 3                  |

were added 13 parts of fine copper bronze. In the absence of inhibitor the resulting composition gelled in a few hours. Upon adding 0.4% of malonic acid (based on the clear lacquer) to the composition, it remained fluid after aging it for a month, while a similar test with malic acid substituted for the malonic acid showed partial gelation at the end of one month.

Although the examples refer solely to the treatment and testing of clear lacquers and lacquers containing various metal powders or pastes, the methods of this invention are also applicable to lacquers containing other forms of pigment, whether packaged in lead or lead-lined containers or otherwise. In general, the most difficult problems of gelation occur with lacquers containing copper-containing or lead-containing powders or pastes of the type referred to in the examples, but the advantages of the invention are also applicable to other types of lacquers, particularly when they are packaged in lead or lead-lined containers.

Where reference is made herein and in the appended claims to bronze powder, it is to be understood that this includes metal powder or flake of such materials as brass, aluminum, lead or copper, and the usual copper-tin or copper-zinc alloys. In some instances, reference is made to metal pastes. These are merely mixtures of metal, i. e. bronze powder with suitable organic solvents, and in some instances, with a polishing or leafing agent, such as stearic acid.

Although the reason for the beneficial action of malonic acid upon lacquers of the type described is not definitely known, it is believed the malonic acid functions as a preventive of gelation by causing the formation of a thin protec-

tive film of insoluble metal malonate on the surface of the metal in contact with the lacquer. This film stifles further corrosion and prevents the building up of a concentration of dissolved metal ions capable of reacting with the nitrocellulose to form the material causing gelation. For example, dissolved lead salts, such as lead naphthenate, react instantly with a nitrocellulose solution to form a gel. Copper salts, on the other hand, do not so react, but instead require the presence of metal powder to cause gelation. Whatever the cause of gelation, however, it is believed the malonic acid functions by virtue of its ability to form a metal malonate which is insoluble in the lacquer solution.

What I claim is:

1. A substantially non-gelling nitrocellulose lacquer containing from 0.01 to 5% by weight of malonic acid based on the total weight of the lacquer prior to the addition of said acid, said lacquer having a tendency to gel in the absence of said acid.

2. A substantially non-gelling nitrocellulose lacquer containing from 0.05 to 1% by weight of malonic acid based on the total weight of the lacquer prior to the addition of said acid, said lacquer having a tendency to gel in the absence of said acid.

3. A substantially non-gelling nitrocellulose lacquer containing nitrocellulose, a solvent mixture, metal powder, and from 0.01 to 5% by weight of malonic acid based on the total weight of the lacquer prior to the addition of said acid, said lacquer having a tendency to gel in the absence of said acid.

4. A substantially non-gelling nitrocellulose lacquer containing nitrocellulose, a solvent mixture, metal paste, and from 0.01 to 5% by weight of malonic acid based on the total weight of the lacquer prior to the addition of said acid, said lacquer having a tendency to gel in the absence of said acid.

5. A substantially non-gelling nitrocellulose lacquer containing nitrocellulose, a solvent mixture, a bronze powder, and from 0.01 to 5% by weight of malonic acid based on the total weight of the lacquer prior to the addition of said acid, said lacquer having a tendency to gel in the absence of said acid.

6. A substantially non-gelling nitrocellulose lacquer containing nitrocellulose, a solvent mixture, lead paste, and from 0.01 to 5% by weight of malonic acid based on the total weight of the lacquer prior to the addition of said acid, said lacquer having a tendency to gel in the absence of said acid.

7. The method of preventing or reducing gelation in a nitrocellulose lacquer containing a metal powder of the type tending to cause gelation which comprises adding to said lacquer from 0.01 to 5% by weight of malonic acid based on the total weight of the lacquer.

8. The method of preventing or reducing gelation in a nitrocellulose lacquer containing a metal paste of the type tending to cause gelation which comprises adding to said lacquer from 0.01 to 5% by weight of malonic acid based on the total weight of the lacquer.

9. The method of preventing or reducing gelation in a nitrocellulose lacquer which is packaged in a lead or lead-lined container which comprises adding to said lacquer from 0.01 to 5% by weight of malonic acid based on the total weight of the lacquer.

GERALD R. BARRETT.